

March 23, 1937.

C. R. ECKERT

2,074,684

PROCESS OF MAKING THICK BUTT SHINGLES

Filed Nov. 25, 1931

2 Sheets-Sheet 1

Fig. 7.



Fig. 10.



Fig. 11.



Fig. 12.



Fig. 13.



INVENTOR

Clarence R. Eckert  
BY *Johns Shingle*  
ATTORNEY

March 23, 1937.

C. R. ECKERT

2,074,684

PROCESS OF MAKING THICK BUTT SHINGLES

Filed Nov. 25, 1931

2 Sheets-Sheet 2

Fig. 3.



Fig. 4.



Fig. 5.



Fig. 2.



Fig. 6.



Fig. 8.



Fig. 9.



INVENTOR

Clarence R. Eckert

BY

Fabis Silby  
ATTORNEY

## UNITED STATES PATENT OFFICE

2,074,684

## PROCESS OF MAKING THICK BUTT SHINGLES

Clarence R. Eckert, Englewood, N. J., assignor to  
The Barrett Company, New York, N. Y., a corporation of New Jersey

Application November 25, 1931, Serial No. 577,193

6 Claims. (Cl. 91—68)

This invention relates to flexible composition shingles and processes of making same, and more particularly, to thick butt strip shingles of the felt base type, coated with waterproofing material, surfaced with granular material, and having the tab portions provided with an additional coating of waterproofing material, and a surfacing of granular material.

One object of this invention is to provide a durable thick butt shingle of attractive appearance which may be laid with other like shingles in overlapping courses to impart to the roof or other surface to which they are applied an irregular or hand-made effect. Another object is to provide an efficient and economical process of making such shingles. Other objects and advantages of this invention will appear from the following detailed description, taken in connection with the accompanying drawings, in which

Fig. 1 is a fragmentary side elevation, somewhat diagrammatic in character, indicating the steps involved in the formation of the thick butt shingle of this invention;

Fig. 2 is a fragmentary plan view of a coated and surfaced felt base, prior to the cutting thereof into strip shingles;

Fig. 3 is a plan view of a thick butt shingle and illustrates a preferred embodiment of this invention;

Fig. 4 is a vertical section through a tab portion of the shingle of Fig. 3;

Fig. 5 is a fragmentary plan view of a number of shingles arranged in abutting relationship and in overlapping courses;

Fig. 6 is a plan view of a modified form of thick butt shingle of this invention;

Fig. 7 is a vertical section through a tab portion of the shingle of Fig. 6;

Fig. 8 is a plan view of another modified form of this invention;

Fig. 9 is a vertical section through a tab portion of the shingle of Fig. 8;

Fig. 10 shows a side elevation of the coating roll employed in applying the waterproofing material to form the thick butt shingle of Fig. 3;

Fig. 11 illustrates, in side elevation, the form of coating roll used to apply the waterproofing material in the formation of the shingles of Fig. 13;

Fig. 12 is a fragmentary plan view of a coated and surfaced felt base prior to the cutting thereof and shows another form of thick butt single embodying this invention; and

Fig. 13 is a plan view of two thick butt singles embodying the principles of this invention, the

shingles being arranged butt-to-butt and moved apart from the position shown in Fig. 12.

Referring to the drawings, reference numeral 1 (Fig. 1) indicates the usual felt base made of rag fiber, paper stock, or other fibrous material and thereafter saturated with bituminous material, as is well known in the art. The saturated felt base 1 is passed between the coating rolls 2, 3, the latter of which rotates in a coating bath 4 containing asphalt or other bituminous material. Waterproofing material may also be fed to the coating roller 2, or other form of coating apparatus might be used to coat both sides of the felt base. The coated base passes over guide roll 5, bringing the cementitious coated side under hopper 6 containing granular material, such as crushed slate, rock or other surfacing material. The granular material from hopper 6 is showered by means of the usual distributing roll 7 onto the coated felt base, completely covering the coating.

The thus surfaced base is then passed about roll 8 which serves to partially embed the granular material in the base. The surfaced base then passes under hopper 9' which applies anti-stick material, such as mica dust, to the rear side, rendering this side non-cementitious. In the continued passage of the base 1 about rolls 8 and 9, excess surfacing material falls off therefrom respectively into the hoppers 6, and 9', whence the surfacing material was delivered to the base 1. The sheet then passes over the drying rolls 10 to 15 and from the roll 15 is passed between the pull rolls 16, 17, which may be suitably driven, the pull rolls 16 rotating at a slightly greater peripheral speed than the rolls 17 to provide a slack of material between the rolls 16 and 17. From the rolls 17, the coated and surfaced strip is fed to a coating appliance indicated generally by the reference numeral 18.

Coating device 18 may consist of a tank 19, having rotatably mounted therein a coating roll 21 of special construction. This roll is designed to apply coating material, such as asphalt or other bituminous waterproofing composition to selected spaced areas of the felt base. The size and shape of the selected areas may be varied to produce shingles having tabs or individual shingle-simulating portions of various shapes and of different lengths and/or widths. In the embodiment of the invention shown in Fig. 10, a coating roll having series of spaced platen portions 22 is employed. The platen portions 22 are disposed in parallel rows which run both longitudinally and circumferentially of the roll.

The individual platens 22 in each circumferential row, indicated by the reference numeral 23, are preferably identical in shape. The individual platens in each longitudinal row, indicated by 5 the reference numerals 24, are of different widths, of the same length, and are spaced different distances apart. In the embodiment shown in Fig. 10, intermediate platen 25 is the widest, platens 26, adjacent to platen 25, are of materially less width than platen 25. The left hand end platen 27 is of somewhat less width than the platen 26 adjacent thereto and the right hand end platen 27 is of somewhat greater width than the platen 26 adjacent thereto. Passage 15 of the surfaced sheet over the coating roll shown in Fig. 10 results in application of the waterproofing material on selected spaced areas arranged in transverse rows 28 of the sheet, as indicated in Fig. 2, the individual areas of each 20 row being of the same length but of different widths, and spaced different distances apart.

If it is desired to produce a shingle such as 25 shown in Figs. 12 and 13, a form of coating roll such as depicted in Fig. 11 is employed. This roll involves two sets of platens arranged longitudinally of the axis of the roll, the sets being diametrically opposite each other. Each set comprises individual platens 31, 32, 33, 34, of the 30 shape shown and separated by slots which may be of the same or different widths. Application of the coating material by means of the coating roll of Fig. 11 results in the formation of parallel transverse spaced bands 35 of coating material on the sheet as shown on Fig. 12, each band being composed of spaced selected areas of the peculiar shape shown in Fig. 12.

From the coating appliance 18, the coated sheet passes over roll 36 and is thus reversed to bring the additionally coated portion under the 40 hopper 37. Granular material, such as crushed slate, preferably of a color contrasting with the color of the granular material in hopper 6 is supplied to hopper 37. If it is desired to make adjacent tab portions of the shingle of different 45 colors, partitions may be inserted in hopper 37 and different colored granular material supplied to the different compartments of the hopper. Granular material is showered from hopper 37 by means of the usual distributing roll 38 onto 50 the coated sheet below. The granular material adheres only to the cementitious coated portions and does not adhere to the portions of the base between the transverse coated stripes or to the uncoated portions between the selected coated 55 areas constituting the transverse coated bands or stripes. From the surfacing hopper 37, the sheet having the granular material thereon passes around roll 39, which functions to partially embed the granular material in the coated portions.

From roll 39 the sheet passes over reversing roll 41. The surfaced sheet in its passage about roll 41 causes the excess granules to fall from the sheet back into the hopper 37. The sheet 60 then passes over drying rolls 42, 43, 44, and 45, and thence to the cutting rolls 46, where it is cut into shingle elements.

In the form of invention shown in Fig. 2, the 70 base 1 having transverse rows 28 may be cut on a line intersecting the forward edge of the transverse bands, as indicated by the reference numeral 53. The shingle shown in Figs. 3 and 4 is thus formed. This shingle is composed of a felt base 54, provided with a seal back coating 55

rendered non-cementitious by the application of mica dust 56 thereto. The face of the element is substantially completely covered by coating 57, which is surfaced with granular material 58. A second coating 59 covers spaced selected areas of the portion of surfacing 58 intended to be exposed, leaving uncoated tab-defining depressions or slots 61 between these areas. As shown in Fig. 3, the spaced selected areas differ in width and are separated by slots of different 10 widths. A second surfacing 62 of granular material is partially embedded in the coating 59.

In lieu of cutting along the line 53, the base of Fig. 2 may be cut along lines 65, which are spaced a slight distance from one transverse edge of the transverse bands 28. The shingle element shown in Figs. 6 and 7 is thus produced. This element differs from that of Figs. 3 and 4 in that it has along the upper edge a narrow elevated or thickened portion 66. This thickened portion is composed of an overlay coating 67 covering the surfacing 57 and a surfacing of granular material 68 partially embedded in coating 61. The upper thickened edge 66 is of substantially the same thickness as the forward tab edge of the element and cooperates therewith to provide a horizontal plane support for the overlying portion of the overlapping element.

The base of Fig. 2 may be cut transversely 30 along lines indicated by the reference numeral 69 to form the strip shingle shown in Figs. 8 and 9. This differs from that of Fig. 3 in that it has, at the forward thickened edge, an integral thin portion 71 which is disposed the full length of the 35 element. The portion 71, when the elements are laid in overlapping courses, accentuates the thickness of the thickened portion of the element to the observer.

Employing the coating roll of Fig. 11 results in 40 the formation of rows 35 composed of selected spaced areas, each having a double coating and surfacing alternating with transverse portions 72 composed of the felt base having a single coating and surfacing thereon. As indicated in Fig. 12, the coated and surfaced base may be cut transversely along lines 73, intersecting the base substantially midway between the thickened portions to form the upper thin end 74 of the elements. The base is also cut transversely along 45 staggered lines 75 to form thickened tabs of different lengths. The differences in the lengths of the tabs are such that, as indicated in Fig. 13, the elements may be placed tab-to-tab, with the forward edge of the longest tab of one shingle abutting against the forward edge of the shortest 50 tab of another like shingle, the forward edges of the other tabs of the two shingle strips also abut. If desired, the base material between the tabs may be removed so that the tabs of different 55 lengths and widths are separated by slots 76.

The shingles are preferably arranged in overlapping courses as shown in Fig. 5. The elements of each course may be laid in abutting relation or in slightly spaced relation so as to form a slot between contiguous shingles. The overlying course of elements is preferably laid with the forward edges 78 overlapping the upper edge 79 of the thickened portion of the underlying elements. Hence, the forward thickened edge of each element is exposed to view and the shingle 70 imparts to the observer an appearance of thickness and solidity.

It will be noted that the shingle of this invention involves no waste in its manufacture. Further, a simple transverse cutting knife only is 75

necessary to produce the same, and while it resembles in appearance the usual strip shingle having tabs separated by slots, slot cutting knives and mechanism for removing the material cut out 5 to form the slots are not necessary for the manufacture of this shingle. Owing to the differences in shape and dimensions of the exposed selected areas of each element, the shingle of this invention avoids the drab and monotonous appearance 10 of existing strip shingles and imparts a variegated, hand-made, or thatched effect to roofs or other surfaces to which they are applied.

As an alternative method, I may omit the first mineral surfacing operation carried out with the 15 hopper 6 and distributing roll 7, surfacing with grit only the limited thick areas resulting from the operation of the roll 21 by means of hopper 37 and distributing roll 38. If I operate in this manner, I find it advantageous to coat the upper 20 surface of the web leaving roll 5 with an anti-sticking material such as a film of soap solution, which will prevent the sheet from sticking to the rolls, but will not prevent the asphalt pads of roll 21 from applying asphalt to the sheet in 25 spaced selected areas. The exposed tab portion of shingles made by this alternative process have substantially the same appearance as those previously described, but the shingles lack the surfacing 30 having in lieu thereof a coating of anti-stick or non-cementitious material.

While preferred embodiments of the invention have been described herein, it will be understood that this invention is not confined to the forms disclosed but may be variously embodied within 35 the scope of the appended claims.

**I claim:**

1. A process of making thick butt shingles which comprises coating substantially the entire surface of an unslotted flexible base with waterproofing material, applying an additional coating 40 of waterproofing material to the coated base, said additional coating being applied in spaced transverse bands, each band consisting of spaced areas simulating individual shingles, separated by portions 45 of the first-mentioned coating left uncovered by said additional coating, and cutting the base transversely to form thick butt shingles.

2. A process of making thick butt shingles which comprises coating substantially the entire 50 surface of an unslotted flexible base with waterproofing material, applying a coating of non-cementitious material to the coated base, applying additional coating of waterproofing material to said non-cementitious coating, said additional 55 coating being applied in spaced transverse bands, each band consisting of spaced areas simulating individual shingles, separated by portions of said non-cementitious coating left uncovered by said additional coating, and cutting the base trans- 60 versely to form thick butt shingles.

3. A process of making thick butt shingles which comprises coating substantially the entire surface of a flexible base with bituminous material, applying an additional coating of bituminous material to selected spaced areas of the first coating 5 said additional coating being applied in transverse bands spaced substantially equal distances apart from each other, each of said bands being composed of selected spaced areas of different widths, connected by portions of the base, and thereafter cutting said base transversely along lines intersecting said selected spaced areas to form thick butt strip shingles.

4. A process of making thick butt shingles which comprises coating substantially the entire 15 surface of a flexible base with waterproofing material, partially embedding granular material in said coating, applying an additional coating of waterproofing material to the partially embedded granular material, said additional coating material being applied in spaced transverse bands, each band consisting of spaced areas simulating individual shingles, partially embedding additional granular material in said additional coating, and cutting the base transversely along 20 lines coinciding with one transverse edge of each of said transverse bands to form thick butt shingles.

5. A process of making thick butt shingles which comprises coating substantially the entire 30 surface of a flexible base with waterproofing material, applying an additional coating of waterproofing material to the coated base, said additional coating being applied in spaced transverse bands, each band consisting of spaced areas 35 simulating individual shingles, and cutting the base transversely along lines substantially midway between said bands and along staggered lines intersecting the said transverse bands to form thick butt shingles having tabs of different 40 lengths.

6. A process of making thick butt shingles which comprises coating substantially the entire surface of a flexible base with waterproofing material, partially embedding granular material 45 in said coating, applying an additional coating of waterproofing material to the partially embedded granular material, said additional coating material being applied in spaced transverse bands, each band consisting of spaced areas 50 simulating individual shingles, partially embedding additional granular material in said additional coating, and cutting the base transversely along lines intersecting the thin portion 55 of the base, spaced somewhat from one transverse edge of said transverse bands to form thick butt shingles having an integral base portion extending from the forward edge of the shingle-simulating portion.

CLARENCE R. ECKERT. 60